

## UNITED STATES PATENT OFFICE

2,103,205

## ART OF SHRINKING FABRICS

Latimer D. Myers, Cincinnati, Ohio, assignor to  
Emery Industries, Inc., Cincinnati, Ohio, a cor-  
poration of Ohio

No Drawing. Application October 19, 1935,  
Serial No. 45,833

15 Claims. (Cl. 26—18.5)

This invention relates to improvements in the art of producing shrunk textiles fabricated from vegetable fibers. More particularly, the invention relates to a process of treating cotton and 5 like fabrics to promote their responsiveness to shrinking operations of the mechanical type. The invention relates also to a material adapted to use in the practice of such process.

In the conventional method of spinning and 10 weaving fabrics, the threads are subjected to tension. This is done to secure proper operation of the spinning and weaving machines and to secure uniformity of weave in the finished product. When only rough fabrics are desired, 15 for example, overall material or denim, the woven textile is often passed directly to a finishing operation wherein it is subjected to treatment with materials adapted to improve, so far as is possible, its "feel", appearance, handle or body. 20 Where fabrics of a better variety are desired, an intermediate step, called "keir boiling", is practiced. It is the function and purpose of this step to remove whatever waxy coating may be present on the fibers and also to 25 remove foreign particles, such as hulls or "shives" by a chemical process of decomposition involving treatment of the fabrics with an alkaline solution under pressure.

In effecting the removal of the waxy impurities and the hulls, the fabrics are rendered more 30 absorbent, permitting them to be uniformly bleached and dyed. After this step is conducted, the fabrics are subjected to a finishing treatment analogous to that previously referred to.

The "finishing" of the fabrics is accomplished 35 by the application of materials such as starches, gums and softeners. These agents are adapted to improve the feel, handle, lustre and general appearance of the fabric. They are generally 40 applied in aqueous solutions in the desired proportions, after which the excess moisture is removed and the fabrics passed through calendar rolls to produce a smooth finish.

Insofar, therefore, as practically all of the 45 textiles of the nature to which the invention relates are woven under tension with the threads in a somewhat stretched condition, fabrics made in such a manner exhibit the tendency to shrink when subjected to water, such as in laundering. 50 A certain degree of shrinkage, of course, does occur in those fabrics which are subjected to keir boiling. Such fabrics, however, again become stretched while being subsequently handled in rope form, while being opened on tentering frames, through pressures applied in passing 55 through finishing calendars and in the various other operations. On the other hand, those fabrics which have not been keir boiled after weaving, comprise threads remaining in the 60 stretched condition in which they are woven.

Shrinkage of these fabrics continues through a number of laundering operations, gradually as the impurities are removed by the soaps and alkalis used in the laundering process.

In either method of manufacture of textiles, 5 in other words, the fibers constituting the finished fabric are in a condition of stress or stretch, and hence tend to shrink under any circumstances that permit or facilitate movement and contraction of the fibers.

A number of methods in the past have been 10 proposed by clothing manufacturers to preclude the shrinkage of fabrics once they are made into garments. The cloth has been subjected to boiling or soaking in water prior to cutting. This 15 method, of course, results in an almost complete loss of the finish previously applied, with the result that the fabric suffers greatly in appearance. Another method adopted by some clothing manufacturers has been to provide an allowance for 20 shrinkage in the cutting of the cloth. The purchaser of such fabrics has great difficulty in obtaining the proper size and has no assurance whatsoever that the shrinkage resulting in subsequent launderings will be uniform in all directions. 25

In recent years it has been proposed to provide 30 a method of treatment that will shrink the fabric in both directions, in a manner analogous to the shrinkage otherwise occurring in the laundering, washing or other cleaning process. This 35 method is predicated upon the determination that the causes of shrinkage in a fabric subjected to full laundry treatment are mostly mechanical in effect. The process is, therefore, adapted to mechanically rearrange the fibers of the fabric to the same extent that these fibers would rearrange themselves if subjected to full laundry washing.

Basically, this process comprises the steps of 40 determining the change in dimension that will take place in the fabric when it is subjected to washing, then mechanically shrinking the fabric down to the shrink dimensions so indicated, and finally completing the finishing operation without disturbing these dimensions. 45

The present invention relates to a process for 50 treating textile fabrics to facilitate shrinking of the fabrics by fiber rearrangement to increase the efficiency and uniformity of shrinkage, and to provide shrink fabrics which are more even 55 and uniform in texture and appearance than the shrink fabrics which heretofore have been available. For the purpose of convenience and illustration, the present invention is disclosed in relation to one particular mechanical method of such preshrinking and to a machine adapted to this process, but the disclosure, in respect to this particular method and machine, is intended only to 60 exemplify the invention, and not to limit it. 60

With the use of the particular machine above referred to, the fabrics, whether they be keir boiled or not, are treated with water solutions or emulsions of materials adapted to enhance their finish, feel and appearance. The excess of finishing agents is removed from the fabrics by passage through squeeze rolls and then whatever moisture is present is removed by drying.

Next, the fabrics are brought to the shrinking machine, preferably in rolled condition. From the roll the material is spread to eliminate wrinkling, then passed on to tentering frames. In the tentering frames a spray of moisture is applied to the fabric on one or both sides. As the material progresses, the tenter stretches the fabrics in width, which results in a lengthwise contraction or shrinkage.

Subsequently, the tenter chains carry the material to a drying chamber where the moisture is driven out. At this point the material has been shrunk in length and stretched in width. Next the fabric leaves the tenter chains, and is subject to moderate predetermined lengthwise tension while a spray of moisture again is applied. This step is effective to cause complete widthwise shrinkage, but also causes a slight elongation of the warp threads. This elongation is compensated by causing the fabrics partially to contract under the influence of heat while being dried and finally finished.

In both warpwise and widthwise shrinkage as carried out in the mechanical process, the degree of shrinkage must be uniform over the entire area of the fabric being shrunk. If it is not so, the threads may be wavy and uneven and tend to distort the fabric or the design on the fabric in case it should previously have been of a printed or woven design.

To summarize briefly therefore, it will be seen that the fabrics, after weaving, first are keir boiled, if desired, then subjected to the finish enhancing materials, and then shrunk in the machine and the finishing operation completed. The shrinking operation must be such as to bring about the desired degree of contraction in the material without defeating or detracting from the finishing agents previously applied to the fabrics. The fabrics going to the machine generally contain all of the materials such as the starches, gums and softeners of various types which are used to improve the finish, these having been applied by a water solution in proper proportion, with the fabric subsequently squeezed to remove the excess and then dried.

Although the fabrics have been wetted by the finishing solutions, it is not feasible to attempt shrinking while in this state as the drying methods which must be employed in order to prevent elongation of the fibers are not adapted for the removal of large quantities of water. For this reason the fabrics are first dried, then moistened with small amounts of water in the shrinking machine, the water subsequently added in these small quantities having the function of rendering the fabrics soft and pliable in order to permit shrinkage. These small amounts of water, approximately 15% more or less by weight, must be distributed and received evenly and uniformly throughout the entire fabric.

It is the object of this invention to provide a process adapted to render such fabric uniformly responsive to the reception of the moisture used in the shrinking process, and to provide a process used in conjunction with the mechanical

shrinking process, adapted to improve the feel and appearance of shrunk fabrics, and at the same time improve the properties of the fabrics shrunk with respect to their stability under unusual atmospheric influences during storage. 5

Another object of the invention has been to treat textile fabrics prior to mechanical pre-shrinking to facilitate shrinking of the fabrics evenly and uniformly during mechanical pre-shrinking. 10

Briefly, the present invention is predicated upon a series of discoveries, concepts and determinations which have required commercial verification. The first of these is that oil soluble mineral oil sulphonates either alone, or combined in varying proportions, possess the capacity to cause fabrics to shrink evenly and uniformly when the fabrics are moistened and then subjected to a process for rearranging the textile fibres mechanically. 20

In view of the fact that it has not been practical in the conventional mechanical preshrinking process to saturate the fabrics thoroughly, prior to mechanical treatment, water usually has been applied in the form of vapor or mist as by spraying. While it is feasible to apply the moisture to the fabric evenly and uniformly, still the fabric itself does not respond evenly to the treatment because of the variations in the absorbency of the fabric from section to section, or from yard to yard being shrunk. 25

However, I have discovered that oil soluble mineral oil sulphonates with or without mineral oil are incorporable in the sizing bath in which the fabrics usually are immersed before being shrunk. During sizing, the sulphonates (and oil if present) are incorporated in the fabric, and finally, when the dried fabrics are remoistened for shrinking, the moisture which is applied uniformly, is distributed and received by the fabrics so that the amount of shrinkage is uniform, and the texture of the shrunk pieces is similar from piece to piece. 35

The oil soluble mineral oil sulphonates, either alone or combined in various proportions with stable mineral oils, improve the appearance of the finished fabrics in which these materials are present. In this respect the fabrics are improved by acquiring an evenness and uniformity of appearance and by exhibiting improved qualities of handle and feel; that is to say, they are appreciably softer and more pliable but with good body. 40

Briefly, the process aspect of the invention resides in the treating of the fabrics with solutions comprising oil soluble mineral oil sulphonates, either alone or in conjunction with stable mineral oils, before such fabrics are shrunk, and, preferably, at the same time that the fabrics are subjected to treatment with the usual finishing agents such as starches, gums, etc., as may be desired. Then the fabrics are passed through squeeze rolls to remove excess quantities of the solutions applied, dried, and passed to the machine or operation effective to accomplish shrinkage of the fabric. 50

The mineral oil sulphonates referred to are derived from the process of producing medicinal white oils and the light-colored technical oils by treating a mineral oil with fuming sulphuric acid and/or sulphur trioxide. As a result of this treatment two layers are formed. The upper layer, known as the A or oil layer, and the lower layer, known as the B layer or sludge layer. The sulphonates of the A layer are highly oil 70 75

soluble. The sulphonates of the B layer are highly water soluble.

I prefer to use A layer or oil soluble sulphonates in this process. However, it may be mentioned in this respect that oil soluble sulphonation products derived from brown coal tar oil may also be used in certain instances in the practice of the present invention.

While any stable chemically inert mineral oil can be used in this process, I prefer to use the white oils or light-colored technical oils produced when lubricating stock or mineral oil is treated with fuming sulphuric acid or sulphur trioxide. This oil, when combined with the oil soluble or A layer sulphonates, becomes readily water soluble, and possesses fine qualities as a fabric softening agent. Less highly refined oils may be used in treating lower grades or dark-colored fabrics, but whatever type of oil is selected for use, its boiling point should be sufficiently high to avoid loss by evaporation.

In general, the quantity of oil—oil soluble mineral oil sulphonate blend used may vary from about .5% to about 7.5% of the weight of the finishing solution to which it is added. In this respect it should be understood that the quantity or proportion and nature of the other finishing agents present in the solution may modify or alter substantially the percentages capable of being used.

When mineral oil is used in conjunction with mineral oil sulphonate, the proportions of the two may vary over a considerable range. For example, where unboiled overall material is to be shrunk, an appreciable quantity, for example as high as 75%, of mineral oil sulphonate in the blend may be advisable, the amount used being determined by that proportion which will dissolve readily in water. On the other hand, for a fabric such as white shirting material, the proportion of mineral oil—oil soluble sulphonate composition, may be as high as 90%. In this latter instance, the quantity and ratio of mineral oil sulphonate to mineral oil is predicated primarily upon the particular finish desired on the fabric.

I may mention that the B layer or water soluble sulphonates possess a number of attributes of the A layer sulphonates but are not as desirable as the latter for the reason that they are generally possessed of relatively dark colors and do not blend well with oils.

The shrinking operation is the final processing operation in the production of the fabrics of the type of cotton. All materials applied previously to the fabric necessarily must remain since in the latter process nothing is removed. Mineral oil sulphonates—mineral oil blends remaining in the fabrics add greatly to the desired fabric properties. Such blends, when compounded with stable white oils, do not become rancid or tend to cause yellowness in storage or upon extended exposure to the atmosphere.

In many instances and especially where fabrics of high quality and fine grade are being manufactured, it may be desirable to use mineral oil sulphonates from which extraneous impurities have been removed, this improving their properties. When this is the case, the sulphonates are readily purified according to the process described in the Fischer-Reddish U. S. Patent No. 1,703,838 and in the Heckel-Reddish U. S. Patent No. 1,775,622.

There are certain instances when a textile manufacturer desires to process a high grade

fabric and to provide it with an extremely soft body and special finish. In these instances it may be desirable to use a fatty body such as the sulphonation products of castor and olive oil, fatty acids and tallow, the soaps of such fats or the fats themselves in conjunction with the sulphonate or sulphonate mineral oil mixture. It should be noted, however, that fatty substances almost always are subject to the criticism that they tend to rancidify during extended storage. When fatty bodies are used in the treating of fabrics to improve appearance, it is advisable that conditions should be such that the fabric so treated will be used after a relatively short period of time.

In the process of the present invention the oil soluble mineral oil sulphonates and the mineral oil promote even distribution and reception of the moisture over the entire area of and throughout a given piece of fabric, whereby waviness or distortion of weave or pattern is eliminated; of rendering soft and pliable the other finishing agents added to the fabric, and improving the feel, appearance, luster and without impairing the normal storage qualities of the fabric so treated.

To assist the skilled in the art in carrying out the process on varieties of fabrics, the following disclosures are provided as examples only:

*Example 1.—Shrinking of denim fabric*

After weaving denim fabric is taken directly from the loom and without being desized or boiled out is padded through a solution containing 100# of a blend of 45% purified oil soluble sulphonate and 55% of pale odorless mineral oil distillate having a viscosity of 80 to 100 sec. at 100° F., and 100# of tapioca starch in 320 gallons of water. The excess solution is squeezed out and the cloth dried. The denim is then passed directly through the shrinking process. The shrinkage is even, uniform and complete. Desizing and boiling out are eliminated with a corresponding reduction in operating costs.

*Example 2.—Shrinking of chambrays*

This material is usually not keir boiled but is lighter in weight than the denims. For shrinking fabric of this type 15# of blend described in Example 1 in 100 gallons of water provides ample wetting. Starches may be added to this solution if desired. In either case the fabric is processed as in Example 1.

*Example 3.—Shrinking white broadcloth and madras*

These materials have been keired and bleached and require less wetting action than un-keired materials but a correspondingly better finish. For this purpose a solution of 25# of a blend of 15% of purified oil soluble mineral oil sulphonates and 85% of white mineral oil dissolved together with 40# of this boiling starch in 100 gallons of water provides an excellent finish agent and ample wetting to insure thorough and uniform shrinkage.

*Example 4.—Treatment of bleached white duck*

This material has also been keired but is a heavy material and is usually given a heavy finish and is therefore more difficult to wet than broad cloths or like fabrics. Fifteen pounds of a blend of 45% purified oil soluble mineral oil sulphonates and 55% of white mineral oil added to the usual finishing solution consisting of 80# 75

of pearl corn starch and 80# of white corn dextrine in 150 gallons of water gives instant wetting by the sprays and results in a completely shrunk fabric.

5 Having described my invention, I claim:

1. In the art of shrinking fabrics mechanically, the step of treating cotton fabrics which are differentially repellent to water, prior to the time that they are shrunk, to render such fabrics uniformly receptive to water in the mechanical shrinking process, which step comprises, treating the fabric to be shrunk with an aqueous solution comprising oil soluble mineral oil sulphonates and stable mineral oil.

10 2. In the art of shrinking fabrics of the type of cotton which are relatively and differentially repellent to water by a process involving the application of water to the fabrics, the step which comprises, padding the fabrics to render them uniformly receptive to water with a solution comprising oil soluble mineral oil sulphonates, and finishing agents, removing the excess of such solution from said fabric, then shrinking said fabric.

15 3. In the art of shrinking fabrics of the type of cotton which are differentially reluctant to receive water by a mechanical process involving the application of water to said fabrics, the step which comprises, rendering the fabrics to be shrunk uniformly receptive to water by treating them, with a solution of finishing agents, containing from about .5 to about 7.5% by weight of said solution of a blend of stable mineral oil and oil soluble mineral oil sulphonates.

20 4. In the art of shrinking fabrics by a process involving the application of water to the fabrics from a spray, the steps which comprise, treating fabrics which are differentially repellent to water with a solution containing stable mineral oil of light color and oil soluble mineral oil sulphonates to render such fabrics uniformly receptive to water, removing the excess of such solution from the cloth, then drying the cloth, and finally passing the cloth so treated to the shrinking operation.

25 5. The process which consists in conditioning a fabric of the type of cotton fabric which is differentially repellent to water in an aqueous solution containing fabric finishing material, and oil soluble mineral oil sulphonates and mineral oil in order to render such a fabric uniformly receptive to water and adapted uniformly to shrink when water is applied to it in a mechanical shrinking process, then removing the excess of aqueous solution from the fabric and drying it, and finally in applying moisture to the fabric and then shrinking it mechanically.

30 6. A process for shrinking fabrics mechanically which includes the step of conditioning those fabrics which are differentially and relatively water repellent to render such fabrics uniformly receptive to moisture by incorporating oil soluble mineral oil sulphonates and mineral oil in such fabrics prior to the time they are shrunk mechanically.

35 7. A method for shrinking fabrics relatively and differentially moisture repellent to render the fabric uniformly affinitive for moisture in a process of shrinking the fabrics mechanically, which method includes the step of treating the fabrics prior to shrinking with an aqueous solution containing oil soluble mineral oil sulphonates and mineral oil.

8. In a process for shrinking fabrics mechanically the method of conditioning fabrics differentially affinitive to moisture to render the fabrics uniformly receptive to moisture which method comprises incorporating in the fabrics evenly and uniformly a blend of oil soluble mineral oil sulphonates and mineral oil.

9. A process of conditioning fabrics of the type of cotton denim which has not been kier boiled and which are differentially and relatively moisture repellent, so that they will receive moisture uniformly in a process of shrinking the fabrics mechanically which method includes the step of incorporating oil soluble and mineral oil sulphonates and mineral oil in such fabrics and then shrinking them mechanically.

10 10. In the art of shrinking fabrics mechanically a process for conditioning fabrics differentially and relatively water repellent to render the fabrics uniformly receptive to moisture which process comprises treating the fabrics in an aqueous solution containing oil soluble mineral oil sulphonates and mineral oil, removing the excess of aqueous solution from the fabrics and drying them, applying moisture uniformly to the fabrics and then shrinking them.

15 11. The method of conditioning a fabric which is differentially reluctant to receive water so that that fabric may be shrunk evenly and uniformly in a mechanical process of shrinking, which involves the application of water to the fabric prior to shrinking, which method consists in treating the fabric in an aqueous solution containing oil soluble mineral oil sulphonates and mineral oil after the fabric has been woven but before it is shrunk, and then in removing the excess of such solution from the fabric and drying it.

20 12. A method of treating woven textile cloth which has a varying affinity for water, in different sections of the cloth in order to render such a cloth evenly and uniformly shrinkable in a mechanical process for shrinking the cloth, which method consists in incorporating oil soluble mineral oil sulphonates and mineral oil into the cloth and then in shrinking it mechanically.

25 13. A method for treating a web of textile cloth which varies in its reluctance to receive water in different sections of the cloth in order to render that cloth uniformly receptive to water and uniformly shrinkable in a mechanical shrinking process, which method comprises, incorporating finishing agents and oil soluble mineral oil sulphonates and mineral oil into the cloth, and then shrinking it mechanically.

30 14. In a process for shrinking fabrics by adding water to them and then shrinking them mechanically, the improvement which consists in treating those fabrics relatively and differentially reluctant to receive water by incorporating oil soluble mineral oil sulphonates and mineral oil into them prior to the time that they are shrunk whereby such fabrics are rendered uniformly shrinkable when water is applied to them and they are shrunk mechanically.

35 15. A process for treating fabrics not possessing the capacity to shrink evenly and uniformly in a mechanical process of shrinking in which water is applied to the fabrics, the improvement which consists in incorporating oil soluble mineral oil sulphonates and mineral oil into such fabrics prior to the time that they are shrunk, and then in shrinking them.

LATTIMER D. MYERS.